

May 22, 1923.

1,456,088

P. A. E. ARMSTRONG

HEAT TREATED STABLE SURFACE ALLOY STEEL

Filed Dec. 12, 1919

TRANSFORMATION CURVE FOR C .40%, Cr 9%, Si 3.50%, Mn .30%, REST PRINCIPALLY Fe



INVENTOR  
P. A. E. Armstrong  
H. H. Dyke  
ATTORNEY

Patented May 22, 1923.

1,456,088

# UNITED STATES PATENT OFFICE.

PERCY A. E. ARMSTRONG, OF LOUDONVILLE, NEW YORK.

## HEAT-TREATED STABLE-SURFACE ALLOY STEEL.

Application filed December 12, 1919. Serial No. 344,294.

*To all whom it may concern:*

Be it known that I, PERCY A. E. ARMSTRONG, a subject of the King of Great Britain, and a resident of Loudonville, county of 5 Albany, and State of New York, have invented certain new and useful Improvements in Heat-Treated Stable-Surface Alloy Steel, of which the following is a specification.

- 10 The present application relates to an alloy steel containing principally iron, chromium, silicon and carbon, in such proportions that, when fixed solid solution ground mass by heat-treatment, it is of 15 stable surface character, that is to say, resistant to change or deterioration, such as produced in ordinary steel, for example, by staining, oxidizing, corroding and the like agents.
- 20 This alloy steel is practically stainless and is resistant to corrosion, oxidation and the like when the ground mass is fixed solid solution by heat-treatment, but is more or less readily attacked by corroding and the 25 like agents when not in such state.

When the ground mass is fixed solid solution by heat treatment, the alloy steel is not attacked or stained to any considerable extent by nitric acid, nor by acetic or other 30 organic acids, fruit juices or the like. It is attacked to some extent, however, by hydrochloric acid, sulfuric acid and hydrofluoric acid, particularly when the acids are diluted.

- 35 The heat treatment of this alloy steel may be of various sorts, so long as same results in fixing the ground mass of the material substantially solid solution. For example, the material may be heated to a high heat, 40 say about 1850°-1900° F., and cooled rapidly in the air, or quenched in molten salts, oil, water and other suitable quenching agents. The constituents making up the major portion or ground mass of the steel appear to 45 be in solution at about the temperatures stated and to be fixed or rendered solid in such solution by the rapid cooling. Normalizing of the crystalline structure of the material, as by slowly cooling, or by long 50 continued annealing or other equivalent normalizing treatment, is to be avoided, if the material is to have good stable surface qualities.

The alloy steel has over about 5% and 55 under about 13% silicon and chromium, taken together. Its stable surface qualities,

while fairly good at or toward such lower limits, are better at or toward the upper limits stated. The upper limit beyond which the material does not require heat treatment, to get desirably good surface stability, cannot be fixed at precisely 13%, but same is at or about the neighborhood of 13% of chromium and silicon, taken together.

The silicon content may be from .5% to 7% and the chromium from 3% to 10%, the proportions being distributed between the chromium and silicon so as to keep the total of silicon and chromium, taken together, between about 5% and about 13%. With such proportions of silicon and chromium, taken together, the carbon should be kept low to get good results. Carbon as low as .05% may be used. Preferably the 75 carbon should be kept under one-half of the silicon when taken alone, and under one-tenth of silicon and chromium, taken together.

With an alloy steel at about the lower end of the range referred to, containing silicon 2.5% and chromium 3%, for example, the carbon should preferably be under .55%, since, with such material, further increase of carbon, to say 1%, results in a considerable reduction of the desired surface stability in the alloy steel. Carbon .30%, for example, gives good results with these proportions of silicon and chromium, provided the ground mass is fixed solid solution by 90 heat treatment.

One good stable surface alloy steel at about the upper end of the range referred to contained silicon 3.7%, chromium 8.9%, carbon .46%, manganese .23%, sulphur .014%, phosphorus .018% and the remainder iron. Substantially as good results may be obtained with more or less variation from these figures, using chromium about 8 to 9%, silicon about 3.50 to 4%, and carbon about .40 to .60%.

The proportions given herein are by weight. It is to be noted that the specific gravity of silicon being only about one-half that of chromium or iron, the percentages of this component, when given by volume instead of by weight, are about twice the figures given herein.

My improved alloy steel, containing substantial proportions of silicon, has greater 110 surface stability, that is to say, is much more resistant to stain, oxidation, corrosion

and the like, than similar material not containing a substantial proportion of silicon.

With the use of silicon as described, a substantially homogeneous and readily workable alloy is obtained. The beneficial action of silicon is not appreciable where it is present only in small proportions, say up to about .30-.40%. To get the beneficial effects desired, at least .50% of silicon must be present, and more silicon is desirable. With the use of silicon as described herein, it becomes possible to have the ground mass of the material substantially solid solution. The more the ground mass is solid solution the greater appears to be the stability of the alloy steel produced. With the silicon in the alloy steel a greater proportion of carbon can be used than would be available for production of stable surface material without a substantial proportion of silicon.

The material has quite distinctive cooling and heating curves showing two marked transformation points or stages, the upper one of which tends to rise with increase of silicon and chromium content or with increase of silicon content alone. In the accompanying drawing I have shown for illustration an approximate curve for material containing chromium 9%, silicon 3.5%, carbon .4%, manganese .3% and practically all the remainder iron. The alloy steel may be used in the cast form, if desired, but, when the silicon is under about 5%, it is specially well adapted for mechanical working. It has a plastic range the length of which is increased with increase of chromium and silicon content, and does not become molten until a temperature is reached above the temperature at which it will subsequently solidify. When cast into small molds it readily solidifies into coherent ingots, which can be worked to good advantage. When cast into larger molds the period of solidification is quite long unless provision is made for withdrawing the heat fairly rapidly. Pouring rapidly, as, for example, through a large nozzle has been found to be of advantage in casting operations, and this is particularly useful when heat is withdrawn by permitting the molten metal to stand in the ladle and then pouring at a temperature well down toward the solidification temperature of the metal.

My improved alloy steel, of course, contains small proportions of metalloids, such as sulphur, phosphorus, etc., and may contain variable percentages of metallic elements, substantially all of which may be present, to some extent, at least. If the chromium-silicon content is relatively high, that is to say, in the neighborhood of 13%, the proportion of metallic elements which may be present without substantial detriment to the surface stability of the alloy steel may be correspondingly increased. It

is undesirable ordinarily with the alloy of the present invention to include any of these metallic elements in percentages over 1% when the total chromium and silicon used is as low as 5%, but when say 13% of chromium and silicon is used, other metallic elements can be incorporated up to a total of about 2% to 5% without a substantial detriment to the valuable properties of my alloy steel. I may, for example, incorporate with the alloy steel having chromium-silicon content of 13%, as much as 4% of cobalt or nickel, 1% of manganese, molybdenum, tungsten, vanadium, titanium, zirconium, or other metals which form silicides or compounds or alloys with the iron, or chromium or both, or which do not materially affect the fixation of solid solution ground mass by heat treatment, with no considerable detriment resulting from their use.

The alloy steel herein described and claimed affords an extremely useful and relatively inexpensive material for making various heat treated products and articles, such as cutlery, tools, etc., which should desirably have good stable surface qualities, but which are not ordinarily to be subjected to the most extreme exposure to staining, oxidizing, corroding and the like agents. Valves and valve seats for internal combustion engines when made from such material, particularly at about the upper end of the chromium and silicon range, stand up over very long periods without regrinding, and the material may be made use of in numerous other ways.

I claim:

1. An alloy steel of substantially high surface stability, having the ground mass fixed substantially solid solution by heat treatment, containing chromium about 3% to 10%, silicon about .5% to 7%, chromium and silicon together about 5% to 13%, carbon over about .05% and under 1/10 of the chromium and silicon taken together, and the principal portion of the remainder iron.

2. An alloy steel of substantially high surface stability when heat treated by heating to about 1850-1900° F. and cooling, containing chromium about 3% to 10%, silicon about .5% to 7%, chromium and silicon, taken together, about 5% to 13%, carbon about .05% to 1.3%, and the principal part of the remainder iron.

3. An alloy steel of substantially high surface stability when cooled down from a high temperature, containing silicon over about .5% and under about 7%, chromium over about 3% and under about 10%, silicon and chromium taken together over about 5% and under about 13%, carbon over about .05%, and under one-tenth the chromium and silicon taken together, and also under one-half the silicon, and the principal part of the remainder iron.

4. An alloy steel of high surface stability when cooled down from a high temperature containing silicon about 3.7%, chromium about 8.9%, carbon about .46% and the principal part of the remainder iron.

5. A heat-treated article of substantially highly stable surface character made from alloy steel containing chromium about 8 to 9%, silicon about 3.50 to 4%, carbon about .40-.60%, and the principal part of the remainder iron.

6. An article of substantially highly stable surface character made from alloy steel having the ground mass fixed substantially solid solution by heat treatment and con-

taining chromium about 8 to 9%, silicon about 3.50 to 4%, carbon about .40-.60%, and the principal part of the remainder iron.

7. A cutlery article of substantially highly stable surface character made from alloy steel having the ground mass fixed substantially solid solution by heat treatment and containing chromium about 8 to 9%, silicon about 3.50 to 4%, carbon about .40-.60%, and the principal part of the remainder iron. 25

In testimony that I claim the foregoing, I have hereto set my hand, this 18th day of November, 1919.

PERCY A. E. ARMSTRONG.